

A. KAUFMAN.  
SODIUM CYANID BRIQUET.  
APPLICATION FILED NOV. 7, 1916.

1,262,057.

Patented Apr. 9, 1918.



# UNITED STATES PATENT OFFICE.

ALFONSE KAUFMAN, OF NEW YORK, N. Y., ASSIGNEE, BY MESNE ASSIGNMENTS, TO AIR REDUCTION COMPANY, INCORPORATED, A CORPORATION OF NEW YORK.

## SODIUM-CYANID BRIQUET.

1,262,057.

Specification of Letters Patent.

Patented Apr. 9, 1918.

Application filed November 7, 1916. Serial No. 130,090.

*To all whom it may concern:*

Be it known that I, ALFONSE KAUFMAN, a citizen of the United States, residing at New York, in the county of New York and

5 State of New York, have invented certain new and useful Improvements in Sodium-Cyanid Briquets, of which the following is a full, clear, and exact description, such as will enable others skilled in the art to which

10 it appertains to make and use the same.

This invention relates to articles of manufacture composed of loose or granular material put up in the form of briquets, or blocks, and it also relates to methods of manufacturing such briquets, or blocks, from loose material, and has particular relation to methods and briquets, or blocks, involving a cyanid composition, as sodium cyanid.

One of the objects of the invention is to 20 provide a cyanid composition, such as sodium cyanid, in a condition suitable for convenient transportation, manipulation, and marketing generally, which condition will be such that it will not be materially deleteriously affected by exposure to the atmosphere, and yet will be such that it may be 25 efficiently directly utilized in its chemical relations.

Another object of the invention is the 30 provision of an efficient method of forming cyanid briquets having the features of utility just mentioned and others which will be apparent from the following description.

Other objects will be in part obvious and 35 in part pointed out hereinafter.

The invention accordingly consists in the several steps and the relation and order of one or more of such steps with relation to each of the others thereof, and in the 40 features of construction, combinations of elements and arrangement of parts, which will be exemplified in the process hereinafter disclosed and the construction hereinafter set forth, and the scope of the application of each of which will be indicated in 45 the following claims.

In the accompanying drawing forming part of this specification, wherein similar reference characters refer to similar parts 50 throughout the several views—

Figure 1 is a diagrammatic illustration of an apparatus by means of which certain

parts of the method may be carried out; and

Fig. 2 is a sectional view of a briquet or 55 block.

One of the important requirements of sodium cyanid is that it shall be in a condition to be readily soluble, and one of the important objects of the present invention is 60 to provide a sodium cyanid briquet which shall be readily soluble to an efficient degree, and yet be protected from being rapidly affected by the moisture in the atmosphere, and from rapid decomposition of 65 the cyanid by the  $\text{CO}_2$  gas in the air.

Referring to the specific briquet, or block, herein disclosed, it is composed wholly of sodium cyanid, although it might be composed of other cyanids, or cyanid mixed 70 with other substances. In forming the briquet, first, loose, granular or powdered sodium cyanid is compressed into briquet form, the inner portion of the briquet retaining its original generally granular, 75 though more compact condition so as to be quite porous, and therefore readily soluble. The outer surface of the briquet is provided with a coat more dense than the inner mass, and which is consequently less rapidly solu-

80 ble than the inner portion or mass of the briquet, and is also less rapidly absorbent than the inner mass. This outer coat or coating may be more practically obtained as a second step in the process by subjecting the briquet to a sufficient temperature to fuse the outer surface of the briquet so as to form a film of fused sodium cyanid thereover. The high temperature required should not be continued long enough to fuse 90 the inner mass of the briquet, but only long enough to fuse the outer surface and so that the inner mass will remain unfused. Viewed in one aspect, one of the requirements of the invention will be attained on account 95 of the less porosity of the fused outer surface as compared with that of the inner mass. This coating prevents rapid absorption of moisture and also rapid decomposition of the cyanid by the  $\text{CO}_2$  in the air, 100 and may be made of such thinness as not to seriously lessen rapidity of solubility of the briquet as a whole when compared to the rate of solubility of the porous portion

thereof. In the drawing, the numeral 1 indicates the inner porous portion of a briquet, and the numeral 2 the outer fused coating thereon, the illustration being diagrammatic.

Comporting with the general advantages of the invention, when the briquet is of such a size as to make it desirable to utilize only a portion thereof, or to utilize the briquet in a broken form of ascertained weight or size, the opposite faces of the briquet are provided with weakening indentures, or grooves, 3, which may be embodied in the briquet during the compression of the material thereof into briquet form by the first step of the process. In order that the whole outer surface of the briquet may be provided with the coating referred to it produces to efficiency to simultaneously freely expose the entire outer surface, as far as possible, to the fusing temperature, and to this end one or more faces of the briquet is provided with supporting ribs or projections 4, each of the supporting faces of these ribs or projections being of small area as compared with the full area of the outer surface of the briquet.

In Fig. 1 of the drawing is shown a diagrammatic section of a practical form of furnace, by means of which the outer coating of the briquet may be attained. The numeral 5 indicates supports for a cast iron plate 6 on which is erected a fire brick furnace 7 having a vent 8 and gas burners 9. The numeral 10 indicates thermite slag against which the flame of the burners 9 are directed, and 11 indicates guides or supports, one inside and the other outside the furnace chamber, for guiding and supporting an endless carrier or conveyer 12, this conveyer being adapted to support the briquets 13 and carry them through the chamber of the furnace which will be at a sufficiently high temperature to fuse the outer surface of the briquets and form the coating hereinbefore referred to. The conveyers are provided with nibs or tracks 14, preferably having knife edges, and the ribs 5 of the briquets rest upon the nibs 14 so that the under surfaces of the briquets are supported above the surface of the endless carrier whereby the said under surfaces, as well as the upper and lateral surfaces, are freely exposed to the temperature conditions in the furnace chamber.

The loose or powdered material may be manufactured into briquet form in any suitable compressor, as for instance, in a hydraulic press, the die and platen of which press are designed to give the desired form and size to the briquet as well as to provide the indentures 3, and the supporting-ribs 4.

From the foregoing it will be apparent that the objects hereinbefore referred to, among others, will be efficiently attained.

As many changes could be made in carrying out the above process, and in the above construction, and many apparently widely different embodiments of this invention could be made without departing from the scope thereof, it is intended that all matter contained in the above description or shown in the accompanying drawing shall be interpreted as illustrative and not in a limiting sense.

It is also to be understood that the language used in the following claims is intended to cover all of the generic and specific features of the invention herein described and all statements of the scope of the invention, which, as a matter of language, might be said to fall therebetween.

Having described my invention, what I claim as new and desire to secure by Letters Patent is:

1. A briquet of a cyanid composition having an inner portion and an outer coating, both being of the same chemical composition, but said outer coating being less rapidly soluble than the inner portion.

2. A briquet of a cyanid composition having an inner portion and an outer coating, both being of the same chemical composition, but said outer coating being less absorbent than the inner portion.

3. A briquet of sodium cyanid, comprising an inner portion of compressed sodium cyanid having an outer surface of previously fused sodium cyanid.

4. A briquet of sodium cyanid, comprising an inner portion of compressed sodium cyanid having an outer surface of previously fused sodium cyanid, said briquets having briquet supporting ribs on one face, the supporting faces of said ribs being of small area as compared with the full area of said faces of the briquet.

5. A briquet having an inner porous composition and an outer previously fused surface of less porosity than the inner mass, said outer surface having the same chemical composition as the inner portion.

6. The method of manufacturing briquets which comprises compressing a composition including cyanid into briquet form, and providing said briquet with a coat of the same material which is less rapidly affected by gas and moisture than the inner mass of the briquet.

7. The method of manufacturing briquets which comprises compressing sodium cyanid into briquet form, and providing said briquet with a coat of sodium cyanid of a consistency less rapidly affected by gas and moisture than the inner mass of the briquet.

8. The method of manufacturing briquets which comprises compressing sodium cyanid into briquet form, and providing said briquet with a coat of fused sodium cyanid.

9. The method of manufacturing briquets

which comprises compressing powdered sodium cyanid into a block, fusing the outer surface of said block, and maintaining the inner mass unfused.

5 10. The method of manufacturing briquets, which comprises compressing powdered sodium cyanid into a block and subjecting the same to a temperature at a sufficient height and for sufficient time to fuse the outer sur-

face of the same but not long enough to fuse 10 the inner mass.

In testimony whereof I affix my signature in the presence of two witnesses.

ALFONSE KAUFMAN.

Witnesses:

J. W. ANDERSON,  
C. J. KULBERG.